

## UNITED STATES PATENT OFFICE.

SIDNEY D. WELLS, OF QUINCY, ILLINOIS, ASSIGNOR TO PAPER MILL LABORATORIES, INC., OF QUINCY, ILLINOIS, A CORPORATION OF ILLINOIS.

## PROCESS FOR SOFTENING VEGETABLE FIBERS.

No Drawing.

Application filed September 25, 1926. Serial No. 137,819.

This invention relates to processes for softening vegetable fibrous material, such as wood, cereal straws, and grasses, whereby a remarkably fine product may be obtained by 5 the use of relatively inexpensive chemicals.

The invention includes the feature of relying on sodium carbonate to effect the softening action, as contrasted to a pulping action, all causticizing and dissolving action 10 being avoided.

In my application for patent, Serial 119,471, filed June 29, 1926, now Patent No. 1,626,171, April 26, 1927, entitled Process for cooking vegetable fiber is described an improvement 15 in softening vegetable fibrous materials by the use of sodium carbonate and sulphur and without causticizing the sodium material. The present invention constitutes an improvement over that process of 20 Serial 119,471 in that the sodium carbonate and sulphur are respectively substituted by the materials of spent cooking liquor known, as "black liquor," remaining after fibrous material has been pulped, as contrasted to softened, in the soda process or sulphate process. The liquor, as such, may be used and prior to and dispensing with the refining of 25 the recoverable soda and sulphur content or it may be concentrated and burned and the 30 ash used in subsequently prepared solution. In either case causticizing is avoided.

Heretofore, in the manufacture of paper pulp from vegetable fibrous material such as wood and straw, sodium hydroxide has 35 been frequently used either alone or in the presence of other sodium compounds, such as sodium carbonate, sodium sulphide, sodium sulphite, or sodium sulphate. The sodium hydroxide has been usually relied upon 40 as the major pulping agent, and the other compounds are either present as unavoidable companions from the recovery process or on account of their power to protect the cellulose from the drastic solvent and hydrolytic action 45 of the hydroxide. In the recovery of the sodium salts from the spent cooking liquors, various procedures are used including evaporation and incineration, and smelting is used in the case of the sulphate process. 50 Such recovered soda is largely in the form of sodium carbonate. Losses occur in the recovery of the soda and in the soda process such losses are made up by adding sodium carbonate to the solution of the recovered 55 soda. In the sulphate process, which is to be

considered a modification of the soda process, the losses are made up by adding sodium sulphate to the black ash or black liquor at some point before reaching the smelters. The resultant soda, after leaving the smelters, 60 consists largely of sodium carbonate with certain amounts of sodium sulphide, sodium sulphate, with various other sulphur compounds with sodium and some impurities. The proportions of the essential ingredients 65 in these compounds vary in different mills, depending on their methods of operation. In every case, however, the major portion of the sodium carbonate is converted to sodium hydroxide by means of calcium hydroxide 70 before use in the cooking operation. This conversion or causticizing step is obviated in the present invention.

It has now been found that where only the softening of the vegetable fibrous material is desired, it is not necessary to effect the conversion just mentioned, but soda, such as may be recovered from spent digesting liquors, can be used with whatever sulphur compounds occur, directly in the cooking operation. Where the products obtained may be of a deep brown color, the spent digesting liquor from the complete pulping operation on other material may be used, since much of the soda is in loose combination with weak 85 organic acids or carbonic acid, and is capable of considerable softening action. Spent softening liquor from the process disclosed herein or in my copending application Serial No. 119,471, in which there is provided 90 initial material consisting of sodium carbonate and sulphur, would be of little use, however, on account of its greatly diminished power to soften and reduce. It can be concentrated and incinerated and used the same 95 as incinerated or smelted liquor from soda or sulphate mills as a source of sodium carbonate and sodium sulphur compounds in the preparation without causticizing of a softening solution suitable for the preparation 100 of lighter colored pulp products as disclosed herein. If sodium sulphate be used to make up the loss in recovery or to even partially make it up, no additional sulphur is necessary for the present process. Otherwise sufficient sulphur should be added to the digestors along with the solution of recovered sodium salts and soda ash sufficient 105 to make up the losses to give a desired softening effect.

In conducting the process, the cooking vessels, digestors, are charged with straw or other vegetable fibrous material in the usual manner, together with about sufficient spent 5 digesting liquor to furnish a strength equivalent to seven pounds of sodium carbonate, one pound of free sulphur, similar to the use of free sulphur as in my application Serial No. 119,471, and approximately one hundred 10 dried and seventy pounds of water for every one hundred pounds of straw. The sodium carbonate and sulphur and water are of course not distinct as such since in the spent digesting liquor these materials are more or 15 less in combination with each other and with other materials present. Accordingly the proportions given herein are specified merely to indicate desired strength for treating a given amount of straw, and the qualities 20 of the liquor must be either fairly well known or else it must be analyzed to determine its strength and composition. A cooking treatment of six hours is sufficient if at least five and one half hours of the treatment are conducted at a temperature of 145° C. The action 25 is conducted in closed vessels and at pressures greater than atmospheric. After digestion, the stock is dumped, washed and beaten according to established practice.

30 As an optional treating solution, it has been found that adequate softening may be obtained by using four parts of sodium carbonate and two parts of sodium sulphide for each one hundred parts of straw.

35 The above proportions relate to parts by weight.

Not only may sodium carbonate and sodium sulphide obtained in the recovery operation be used, but they can be purchased and 40 used without recovery.

When straw is used, the steps are substantially the same as in common practice. When wood is used, a mechanical disintegration of the softened chips may be necessary, following 45 the treatment described in my application for patent, Serial 49,461, filed August 10, 1925.

By using the spent digesting liquors described in the foregoing, it will be obvious 50 that time and expense is saved by avoiding the known recovery processes which almost invariably had included causticizing where sodium hydroxide was to be obtained. It is of peculiar importance in the present invention 55 in which the chief aim is to soften and pulping is to be avoided.

The present invention further differs from other processes in that sodium carbonate and sodium sulphide are proposed as cooking 60 agents and with the exclusion of the usual sodium hydroxide which formerly has been used as the principal cooking agent. Sodium hydroxide is far too active an agent for the purpose of merely softening wood, straw, and similar fibrous material without com-

pletely dissolving the non-cellulose material.

It is interesting to observe that there are conditions, circumstances, in which the use of black liquor from the soda or the sulphate processes may be used, and this is where the deep discoloration caused by their use would not be objectionable. It would be necessary to operate the process in conjunction with a plant engaged in making standard soda or sulphate pulp in order to obtain a supply of 70 suitable black liquor. Attention is directed to the fact that the particular spent cooking liquor obtained from the softening operation disclosed in this application and in my application Serial 119,471, would not be effective because in it the soda is a stronger chemical combination and has lost its softening and reducing power, but this liquor, however, can be concentrated and burned just the same as in the soda and sulphate processes and thus 75 the ash may be used as a source of sodium carbonate and sodium sulphur compounds for making up a softening solution desirable 80 where a product as light as possible in color 85 is desired.

90 I claim:

1. In the process of softening vegetable fibrous material, the steps consisting of softening fibrous material by treating it without pulping it with the materials comprising the 95 spent cooking liquors from pulping processes using sodium hydroxide and free from the presence of more powerful chemicals, such materials containing sodium carbonate and being used without further refining and in 100 the presence of sulphur.

2. In the process of softening vegetable fibrous material, the steps consisting of softening vegetable fibrous material without pulping it by treating particles of such material in intermingled contact with the materials comprising the spent liquors from pulping processes and in which sodium carbonate and sodium sulphur mixtures have been used, and conducting such treatment to such an extent as to soften the particles, such materials containing sodium compounds and being used with the fibrous materials to be softened and free from the presence of more powerful chemicals and without causticizing and in 110 the presence of sulphur.

3. In the process of softening vegetable fibrous material, the steps consisting of treating particles of such material in intermingled contact with the sodium carbonate compounds recovered from pulping processes in which sodium carbonate and sodium sulphur mixtures have been used, and conducting such treatment to such an extent as to soften the particles, such sodium carbonate compounds being used with the fibrous materials 120 to be softened and without causticizing.

4. In the process of softening vegetable fibrous material, the steps consisting of treating particles of such material in intermingled 125

- contact with a solution containing sodium carbonate recovered from pulping processes in which sodium carbonate and sodium sulphur mixtures have been used, and conducting such treatment to such an extent as to soften the particles, and using such solutions with the fibrous material to be softened in amounts of solution sufficient to furnish seven parts of sodium carbonate, one part of sulphur and one hundred and seventy parts of water for each one hundred parts of fiber, by weight.
5. In the process of softening vegetable fibrous material, the step consisting of treating particles of such material in intermingled contact with the sodium carbonate solutions recovered from pulping processes in which sodium carbonate and sodium sulphur mixtures have been used, and conducting such treatment to such an extent as to soften the particles, and using such solutions with the fibrous material to be softened in amounts of solution sufficient to provide four parts of sodium carbonate and two parts of sodium sulphide for each one hundred parts of fiber.
10. In the process of softening vegetable fibrous material, the step consisting of treating such fibrous material with a mixture of sodium carbonate and sodium sulphide, said treatment being conducted sufficiently long 30 so as to soften the particles of such fibrous material.
15. In the process of softening vegetable fibrous material, the step consisting of treating such fibrous material with a mixture of sodium carbonate and sodium sulphide in solution, and conducting such treatment to such an extent as to soften the fibrous material, and using such solution in amounts sufficient to furnish seven parts of sodium carbonate, one part of sodium sulphide, and one hundred and seventy parts of water for each one hundred parts of fibrous material, by weight.
20. In the process of softening vegetable fibrous material, the steps consisting of softening fibrous material by treating it without pulping it with the materials comprising the spent cooking liquor from pulping processes and known as "black liquor" and free from 50 the presence of more powerful chemicals and used without further refining and in the presence of sulphur.
25. In the process of softening vegetable fibrous material, the step consisting of treating such fibrous material with a mixture of

35. In the process of softening vegetable fibrous material, the step consisting of treating such fibrous material with a mixture of sodium carbonate and sodium sulphide in solution, and conducting such treatment to such an extent as to soften the fibrous material, and using such solution in amounts sufficient to furnish seven parts of sodium carbonate, one part of sodium sulphide, and one hundred and seventy parts of water for each one hundred parts of fibrous material, by weight.

40. In the process of softening vegetable fibrous material, the steps consisting of softening fibrous material by treating it without pulping it with the materials comprising the spent cooking liquor from pulping processes and known as "black liquor" and free from 50 the presence of more powerful chemicals and used without further refining and in the presence of sulphur.

45. In the process of softening vegetable fibrous material, the steps consisting of softening fibrous material by treating it without pulping it with the materials comprising the spent cooking liquor from pulping processes and known as "black liquor" and free from 50 the presence of more powerful chemicals and used without further refining and in the presence of sulphur.

In testimony whereof I affix my signature.

SIDNEY D. WELLS.